

# United States Patent [19]

Campbell

[11] Patent Number: 4,814,321

[45] Date of Patent: Mar. 21, 1989

[54] **ANTISTATIC LAYER FOR DYE-RECEIVING ELEMENT USED IN THERMAL DYE TRANSFER**

[75] Inventor: **Robert B. Campbell**, Pittsford, N.Y.

[73] Assignee: **Eastman Kodak Company**,  
Rochester, N.Y.

[21] Appl. No.: **123,437**

[22] Filed: **Nov. 20, 1987**

[51] Int. Cl.<sup>4</sup> ..... **B41M 5/035; B41M 5/26**

[52] U.S. Cl. ..... **503/227; 8/471;**  
428/211; 428/331; 428/412; 428/513; 428/913;  
428/914

[58] Field of Search ..... **8/470, 471; 427/146,**  
427/256; 428/195, 206, 323, 331, 480, 913, 914;  
430/200, 201, 945; 503/227

[56]

## References Cited

### U.S. PATENT DOCUMENTS

4,720,480 1/1988 Ito et al. ..... 503/227

### FOREIGN PATENT DOCUMENTS

194106 9/1986 European Pat. Off. ..... 503/227

*Primary Examiner*—Bruce H. Hess  
*Attorney, Agent, or Firm*—Harold E. Cole

[57]

## ABSTRACT

A dye-receiving element for thermal dye transfer comprising a paper support having on one side thereof a polymeric dye image-receiving layer and on the other side thereof an antistatic layer comprising particulate material having a particle size of at least about 2  $\mu$ m.

6 Claims, No Drawings

**ANTISTATIC LAYER FOR DYE-RECEIVING ELEMENT USED IN THERMAL DYE TRANSFER**

This invention relates to dye-receiving elements used in thermal dye transfer, and more particularly to the use of an antistatic layer having particulate material of a certain particle size.

In recent years, thermal transfer systems have been developed to obtain prints from pictures which have been generated electronically from a color video camera. According to one way of obtaining such prints, an electronic picture is first subjected to color separation by color filters. The respective color-separated images are then converted into electrical signals. These signals are then operated on to produce cyan, magenta and yellow electrical signals. These signals are then transmitted to a thermal printer. To obtain the print, a cyan, magenta or yellow dye-donor element is placed face-to-face with a dye-receiving element. The two are then inserted between a thermal printing head and a platen roller. A line-type thermal printing head is used to apply heat from the back of the dye-donor sheet. The thermal printing head has many heating elements and is heated up sequentially in response to the cyan, magenta and yellow signals. The process is then repeated for the other two colors. A color hard copy is thus obtained which corresponds to the original picture viewed on a screen. Further details of this process and an apparatus for carrying it out are contained in U.S. Pat. No. 4,621,271 by Brownstein entitled "Apparatus and Method For Controlling A Thermal Printer Apparatus," issued Nov. 4, 1986, the disclosure of which is hereby incorporated by reference.

In EPA No. 194,106, antistatic layers are disclosed for coating on the back side of a dye-receiving element. Among the materials disclosed for use are electron conductive inorganic powders such as a "fine powder of titanium oxide or zinc oxide".

In U.S. Pat. No. 4,716,145 of Vanier et al. issued Dec. 29, 1987, there is disclosed a technique for reheating dye-receiving elements having transferred dye images in order to drive the dyes deeper into the receiving layer, thereby reducing dye stratification and improving dye stability. One of the ways to accomplish this reheating step is to use a separate heated fusing roller in a print finisher.

A problem exists with using this reheating technique on dye-receiving elements having an antistatic layer on the back. Occasionally by mistake, one of the elements is passed through the print finisher with the back side facing the heated fusing roller (contrary to normal usage where the back side should be away from contact with the heated roller). When this happens, severe fusing of the element to the heated roller occurs and renders the print finisher useless, or at the least requires disassembly and extensive cleaning of the device.

It would be desirable to provide a backing layer for a dye-receiving element which, if by mistake were passed through a print finisher wrong side up, would not stick to the heated roller.

These and other objects are achieved in accordance with this invention which comprises a dye-receiving element for thermal dye transfer comprising a paper support having on one side thereof a polymeric dye image-receiving layer and on the other side thereof an antistatic layer comprising particulate material having a particle size of at least about 2  $\mu\text{m}$ .

Any particulate material may be used in the antistatic layer of the invention provided it has the minimum particle size as noted above. There may be used, for example, silicon dioxide, titanium dioxide or barium sulfate. In a preferred embodiment, silicon dioxide is employed.

It is believed that the relatively large particle size of the particulate material employed in the antistatic layer of the invention provides sufficient surface discontinuities to prevent the overcoat layer from melting and sticking to a heated fusing roller.

In another preferred embodiment of the invention, a polymeric layer is employed between the paper support and the antistatic layer. Any polymeric material may be employed in this layer such as polyolefins like polyethylene and polypropylene, polyethylene terephthalate or polycarbonate.

In another preferred embodiment of the invention, a polymeric layer is present between the paper surface and the dye image-receiving layer. For example, there may be employed polyolefins such as polyethylene, polypropylene, etc. In another preferred embodiment, white pigments such as titanium dioxide, zinc oxide, etc., may be added to the polymeric coating to provide reflectivity. In addition, a subbing layer may be used over this polymeric layer such as a vinylidene chloride copolymer. For example, there may be employed a copolymer comprising from about 5 to about 35 percent by weight of recurring units of an ethylenically unsaturated monomer, from about 0 to about 20 percent by weight of recurring units of an ethylenically unsaturated carboxylic acid, and from about 55 to about 85 percent by weight of recurring units of vinylidene chloride. Further examples of these subbing layers are found in U.S. Pat. No. 4,748,150 of Vanier and Lum issued May 31, 1988.

The polymeric dye image-receiving layer of the dye-receiver of the invention may comprise, for example, a polycarbonate, a polyurethane, a polyester, polyvinyl chloride, poly(styrene-co-acrylonitrile), poly(caprolactone) or mixtures thereof. The dye image-receiving layer may be present in any amount which is effective for the intended purpose. In general, good results have been obtained at a concentration of from about 1 to about 5 g/m<sup>2</sup>.

In a preferred embodiment of the invention, the dye image-receiving layer is a polycarbonate. The term "polycarbonate" as used herein means a polyester of carbonic acid and a glycol or a dihydric phenol. Examples of such glycols are dihydric phenols are p-xylylene glycol, 2,2-bis(4-oxyphenyl)propane, bis(4-oxyphenyl)methane, 1,1-bis(4-oxyphenyl)ethane, 1,1-bis(oxyphenyl)butane, 1,1-bis(oxyphenyl)cyclohexane, 2,2-bis(oxyphenyl)butane, etc.

In another preferred embodiment of the invention, the polycarbonate dye image-receiving layer is a bisphenol-A polycarbonate having a number average molecular weight of at least about 25,000. In still another preferred embodiment of the invention, the bisphenol-A polycarbonate comprises recurring units having the formula



wherein n is from about 100 to about 500.

Examples of such polycarbonates include General Electric Lexan® Polycarbonate Resin #ML-4735 (Number average molecular weight app. 36,000), and Bayer AG Makrolon #5705® (Number average molecular weight app. 58,000). The later material has a  $T_g$  of 150° C.

A dye-donor element that is used with the dye-receiving element of the invention comprises a support having thereon a dye layer. Any dye can be used in such a layer provided it is transferable to the dye image-receiving layer of the dye-receiving element of the invention by the action of heat. Especially good results have been obtained with sublimable dyes. Examples of sublimable dyes include anthraquinone dyes, e.g., Sumikalon Violet RS® (product of Sumitomo Chemical Co., Ltd.), Dianix Fast Violet 3R-FSO® (product of Mitsubishi Chemical Industries, Ltd.), and Kayalon Polyol Brilliant Blue N-BGM® and KST Black 146® (products of Nippon Kayaku Co., Ltd.); azo dyes such as Kayalon Polyol Brilliant Blue BM®, Kayalon Polyol Dark Blue 2BM®, and KST Black KR® (products of Nippon Kayaku Co., Ltd.), Sumickaron Diazo Black 5G® (product of Sumitomo Chemical Co., Ltd.), and Miktazel Black 5GH® (product of Mitsui Toatsu Chemicals, Inc.); direct dyes such as Direct Dark Green B® (product of Mitsubishi Chemical Industries, Ltd.) and Direct Brown M® and Direct Fast Black D® (products of Nippon Kayaku Co. Ltd.); acid dyes such as Kayanol Milling Cyanine 5R® (product of Nippon Kayaku Co. Ltd.); basic dyes such as Sumiacryl Blue 6G® (product of Sumitomo Chemical Co., Ltd.), and Aizen Malachite Green® (product of Hodogaya Chemical Co., Ltd.);

used at a coverage of from about 0.05 to about 1 g/m<sup>2</sup> and are preferably hydrophobic.

The dye in the dye-donor element is dispersed in a polymeric binder such as a cellulose derivative, e.g., cellulose acetate hydrogen phthalate, cellulose acetate, cellulose acetate propionate, cellulose acetate butyrate, cellulose triacetate; a polycarbonate; poly(styrene-co-acrylonitrile), a poly(sulfone) or a poly(phenylene oxide). The binder may be used at a coverage of from about 0.1 to about 5 g/m<sup>2</sup>.

The dye layer of the dye-donor element may be coated on the support or printed thereon by a printing technique such as a gravure process.

Any material can be used as the support for the dye-donor element provided it is dimensionally stable and can withstand the heat of the thermal printing heads. Such materials include polyesters such as poly(ethylene terephthalate); polyamides; polycarbonates; glassine paper; condenser paper; cellulose esters such as cellulose acetate; fluorine polymers such as polyvinylidene fluoride or poly-(tetrafluoroethylene-co-hexafluoropropylene); polyethers such as polyoxymethylene; polyacetals; polyolefins such as polystyrene, polyethylene, polypropylene and methylpentane polymers; and polyimides such as polyimide-amides and polyether-imides. The support generally has a thickness of from about 2 to about 30  $\mu$ m. It may also be coated with a subbing layer, if desired.

A dye-barrier layer comprising a hydrophilic polymer may also be employed in the dye-donor element between its support and the dye layer which provides improved dye transfer densities. Such dye-barrier layer materials include those described and claimed in U.S. Pat. No. 4,700,208 of Vanier et al, issued Oct. 13, 1987.

The reverse side of the dye-donor element may be coated with a slipping layer to prevent the printing head from sticking to the dye-donor element. Such a slipping layer would comprise a lubricating material such as a surface active agent, a liquid lubricant, a solid lubricant or mixtures thereof, with or without a polymeric binder. Preferred lubricating materials include oils or semi-crystalline organic solids that melt below 100° C. such as poly(vinyl stearate), beeswax, perfluorinated alkyl ester polyethers, phosphoric acid esters, silicone oils, poly(caprolactone), carbowax or poly(ethylene glycols). Suitable polymeric binders for the slipping layer include poly(vinyl alcohol-co-butyral), poly(vinyl alcohol-co-acetal), poly(styrene), poly(styrene-co-acrylonitrile), poly(vinyl acetate), cellulose acetate butyrate, cellulose acetate or ethyl cellulose.

The amount of the lubricating material to be used in the slipping layer depends largely on the type of lubricating material, but is generally in the range of about 0.001 to about 2 g/m<sup>2</sup>. If a polymeric binder is employed, the lubricating material is present in the range of 0.1 to 50 weight %, preferably 0.5 to 40, of the polymeric binder employed.

As noted above, dye-donor elements are used to form a dye transfer image. Such a process comprises image-wise-heating a dye-donor element and transferring a dye image to a dye-receiving element as described above to form the dye transfer image.

A process according to the invention of forming a stable dye transfer image comprises heating a dye-receiving element containing a transferred dye image, the dye-receiving element comprising a paper support having on one side thereof a polymeric dye image-receiving layer, and wherein the support has on the



or any of the dyes disclosed in U.S. Pat. No. 4,541,830, 65 the disclosure of which is hereby incorporated by reference. The above dyes may be employed singly or in combination to obtain a monochrome. The dyes may be

other side thereof an overcoat layer comprising particulate material having a particle size of at least about 2  $\mu\text{m}$  as described above.

The dye-donor element employed in certain embodiments of the invention may be used in sheet form or in a continuous roll or ribbon. If a continuous roll or ribbon is employed, it may have only one dye thereon or may have alternating areas of different dyes such as cyan, magenta, yellow, black, etc., as disclosed in U.S. Pat. No. 4,541,830.

In a preferred embodiment of the invention, a dye-donor element is employed which comprises a poly(ethylene terephthalate) support coated with sequential repeating areas of cyan, magenta and yellow dye, and the above process steps are sequentially performed for each color to obtain a three-color dye transfer image. Of course, when the process is only performed for a single color, then a monochrome dye transfer image is obtained.

Thermal printing heads which can be used to transfer dye from the dye-donor elements employed in the invention are available commercially. There can be employed, for example, a Fujitsu Thermal Head (FTP-040 MCS001), a TDK Thermal Head F415 HH7-1089 or a Rohm Thermal Head KE 2008-F3.

A thermal dye transfer assemblage of the invention comprises

(a) a dye-donor element as described above, and  
(b) a dye-receiving element as described above, the dye-receiving element being in a superposed relationship with the dye-donor element so that the dye layer of the donor element is in contact with the dye image-receiving layer of the receiving element.

The above assemblage comprising these two elements may be preassembled as an integral unit when a monochrome image is to be obtained. This may be done by temporarily adhering the two elements together at their margins. After transfer, the dye-receiving element is then peeled apart reveal the dye transfer image.

When a three-color image is to be obtained, the above assemblage is formed on three occasions during the time when heat is applied by the thermal printing head. After the first dye is transferred, the elements are peeled apart. A second dye-donor element (or another area of the donor element with a different dye area) is then brought in register with the dye-receiving element and the process repeated. The third color is obtained in the same manner.

The following example is provided to illustrate the invention.

#### EXAMPLE 1

(A) A dye-receiver was prepared by obtaining a commercially produced paper stock 6.5 mil (165  $\mu\text{m}$ ) thick 40 lb/1000 ft<sup>2</sup> (195 g/m<sup>2</sup>) mixture of hard woodkraft and soft wood-sulfite bleached pulp. The paper stock was then extrusion overcoated with an approximately 1:4 ratio of medium density:high density polyethylene (2.5 lb/1000 ft<sup>2</sup>) (12 g/m<sup>2</sup>) with approximately 6 wt. percent anatase titanium dioxide and 1.5 wt. percent zinc oxide (layer thickness 12  $\mu\text{m}$ ). The support was then coated with the following layers:

- (a) Subbing layer of poly(acrylonitrile)-co-vinylidene chloride-co-acrylic acid (14:79:7 wt. ratio) (0.54 g/m<sup>2</sup>) coated from a butanone and cyclopentanone solvent mixture; and
- (c) Dye-receiving layer of Makrolon 5705 ® polycarbonate (Bayer AG) (2.9 g/m<sup>2</sup>), 1,4-didecoxy-2,5-

dimethoxybenzene (0.38 g/m<sup>2</sup>), and FC-431 ® surfactant (3M Co.) (0.016 g/m<sup>2</sup>) coated from methylene chloride.

The back side of the receiver was extrusion-coated with a non-pigmented, clear, high-density polyethylene layer (3.0 lbs/1000 ft<sup>2</sup>) (14 g/m<sup>2</sup>). On top of this layer was coated a control antistatic layer having particulate material with a relatively small particle size (0.25 g/m<sup>2</sup>). On another sample of the receiver was coated an antistatic layer according to the invention having particulate material with a particle size of 2  $\mu\text{m}$  (1.5 g/m<sup>2</sup>).

#### Control Antistatic Layer:

|                                                                       |                        |
|-----------------------------------------------------------------------|------------------------|
| Cellosize ® QP-4400H Hydroxy ethyl cellulose (Union Carbide)          | 0.007 g/m <sup>2</sup> |
| Ludox AM ® silicon dioxide app. 0.014 $\mu\text{m}$ diameter (duPont) | 0.229 g/m <sup>2</sup> |
| Triton-X 200E ® surfactant (Rohm & Haas)                              | 0.015 g/m <sup>2</sup> |
| (coated from a water and isobutyl alcohol solvent mixture)            |                        |

#### Invention Antistatic Layer:

|                                                                                     |                        |
|-------------------------------------------------------------------------------------|------------------------|
| Gelatin                                                                             | 0.59 g/m <sup>2</sup>  |
| Unitane 520 ® titanium dioxide app. 0.2 $\mu\text{m}$ diameter (American Cyanamide) | 0.38 g/m <sup>2</sup>  |
| Syloid 244 ® silicon dioxide app. 2 $\mu\text{m}$ diameter (Grace Chemical)         | 0.007 g/m <sup>2</sup> |
| 2,7-Naphthalene disulfonic acid Dow Chemical 620 Latex                              | 0.22 g/m <sup>2</sup>  |
| (coated from a water and isobutyl alcohol solvent mixture)                          | 0.24 g/m <sup>2</sup>  |

A dye-donor element was prepared by coating on a 6  $\mu\text{m}$  poly(ethylene terephthalate) support dye layers containing the dyes as identified above (0.77 mmoles/m<sup>2</sup>), and FC-431 ® (3M Corp.) surfactant (2.2 mg/m<sup>2</sup>) in a cellulose acetate propionate (40% acetyl and 17% propionyl) binder (at 1.8 times that of the dye) coated from a toluene, methanol and cyclopentanone solvent mixture. On the back side of the element was coated a slipping layer of the type disclosed in U.S. Pat. No. 4,737,485 of Henzel et al. issued Apr. 12, 1988.

The dye side of the dye-donor element strip one inch (25 mm) wide was placed in contact with the dye image-receiving layer of the dye-receiving element of the same width. The assemblage was fastened in the jaws of a stepper motor driven pulling device. The assemblage was laid on top of a 0.55 (14 mm) diameter rubber roller and a TDK Thermal Head L-133 (No. C6-0242) and was pressed with a spring at a force of 8 pounds (3.6 kg) against the dye-donor element side of the assemblage pushing it against the rubber roller.

The imaging electronics were activated causing the pulling device to draw the assemblage between the printing head and roller at 0.123 inches/sec (3.1 mm/sec). Coincidentally, the resistive elements in the thermal print head were heated at increments from 0 up to 8.3 msec to generate a graduated density test pattern. The voltage applied to the print head was approximately 21 v represent approximately 1.7 watts/dot (12 mJoules/dot).

The dye-receiving element was separated from the dye-donor element. The receiving elements were then passed through a print finisher comprising a set of rollers, one of which was heated in order to fuse the image. In each case, the receiver was inserted wrong side up (the backing layer facing the heated roller). When the receiver with the control antistatic layer was passed

through the print finisher, severe sticking occurred. The roller had to be replaced. However, when the receiver with the antistatic layer according to the invention was passed through, also wrong side up, no sticking occurred. This print was retrievable for passage through the rollers in the correct way.

The invention has been described in detail with particular reference to preferred embodiments thereof, but it will be understood that variations and modifications can be effected within the spirit and scope of the invention.

What is claimed is:

1. In a process of forming a stable dye transfer image comprising heating a dye-receiving element containing a transferred dye image, said dye-receiving element comprising a paper support having on one side thereof a polymeric dye image-receiving layer, the improvement wherein said support has on the other side thereof

an antistatic layer comprising particulate material having a particle size of at least about 2  $\mu\text{m}$ .

2. The process of claim 1 wherein said particulate material is silicon dioxide.

3. The process of claim 1 wherein a polymeric layer is present between said paper support and said antistatic layer.

4. The process of claim 3 wherein said polymeric layer is polyethylene.

5. The process of claim 1 wherein a polymeric layer is present between said support and said polymeric dye image-receiving layer.

6. The process of claim 1 wherein said dye image-receiving layer is a bisphenol-A polycarbonate having a number average molecular weight of at least about 25,000.

\* \* \* \* \*